

## UNITED STATES PATENT OFFICE.

DEMPSEY KEMP DODGE, OF HOUSTON, TEXAS.

## PROCESS OF FORMING COMPOSITE LUBRICANTS.

No Drawing.

Application filed July 11, 1922. Serial No. 574,292.

*To all whom it may concern:*

Be it known that I, DEMPSEY KEMP DODGE, a citizen of the United States, residing at Houston, Harris County, Texas, have invented a certain new and useful Improvement in Processes of Forming Composite Lubricants, of which the following is a full, clear, and exact description, such as will enable others skilled in the art to which it appertains to make and use the same.

My invention relates to the manufacture of composite lubricating oils which are particularly suited for use in internal combustion engines and on the bearings and other movable parts of machinery. It contemplates the treating and mixing of castor oil with mineral oils in such manner as to obtain lubricants of the desired qualities.

An object of the invention is to obtain a lubricant of superior lubricating quality and heavy viscosity.

Another object is to combine the lubricating qualities of castor oil with those of mineral oils and thus cheapen the cost of manufacture and at the same time obtain a better lubricating oil.

In the production of the best grades of high viscosity petroleum lubricants a large amount of filtering and treatment is necessary. For this reason the cost of manufacture of such grades of lubricating oil is much greater than that of the lighter unfiltered, and less valuable grades. I have conceived the idea of mixing with the lighter grades of lubricants, obtained from mineral oil, a small percentage of castor oil of heavy viscosity and thus securing resulting heavy lubricants of superior lubricating qualities at a lower cost.

The process of treating the ingredients of my improved lubricant is not difficult but various elements in the same will vary slightly depending on the quality of the oil and on the kind of apparatus employed.

I may use a grade of castor oil refined to about the extent of the common product sold for medicinal purposes. Such oil contains a certain amount of acids and aldehydes and is not miscible with mineral oils, at least not without the inclusion of some third oil or ingredient or further treatment.

This grade of commercial castor oil is first subjected to treatment in a still under a temperature of from 280° to 325° centigrade at atmospheric pressure until a definite pro-

portion of the acids and aldehydes is distilled off. The volume thus distilled off may be from 4% to 10% of the mass and with the grade of oil stated will be about 6.5% of the whole.

The residue of this distillation is slightly gummy and of light viscosity. It is therefore further treated by heating and blowing with air until the desired viscosity is obtained and the gumminess not greatly increased. Heating the mass or both the mass and the air to between 75° to 150° C. accelerates the operation but is not absolutely necessary. It is found that when thus blown with air the gumminess of the mass will increase very slowly for a period depending upon the quantity of air, the temperature, and the volume of oil treated. When the point of rapid increase in gumminess has been reached, a further blowing will cause excessive gumminess of the oil. The acid number has been found to decrease with this process. The time of treatment to obtain the slight gumminess and desired viscosity will vary with the apparatus, the temperature and the amount of oil, and can be easily determined by test with any particular installation. Using the medicinal grade of oil mentioned, the viscosity of the mass was found to increase from 715" at 100° Fahrenheit Saybolt universal viscosimeter to around 3500" at 100 degrees Fahrenheit by the same method before the mass began to show a marked tendency to increase in gumminess.

This heavy grade of oil is easily miscible with mineral oil and I contemplate using a light, and hence cheap grade of mineral oil lubricant and mixing it with a small percentage of this heavy castor oil product and thus obtaining a lubricant of the required viscosity. The various grades of medium, heavy, and extra heavy lubricating oil may be thus obtained by mixing with the light grades an amount of the heavy castor oil sufficient to produce the desired consistency. This compounded lubricant is preferably made homogeneous by mixing when the mass is heated to from 50° to 150° C. When cool the product is ready for use, and will not separate on standing.

The advantages of my improved lubricant will be obvious to one skilled in the art. The lubricant of desired viscosity can be obtained cheaply and the degree of viscosity desired can be produced by the simple step of

mixing the heavy castor oil product with the cheaper light grades of mineral lubricant in the desired proportions. Grades heavier than those obtainable from pure mineral oils 5 can be produced and the resulting product may be almost colorless. There will be no appreciable tendency to gum or form carbon as may occur with certain heavy lubricants including pure castor oil or lubricants produced by other means. The product is 10 cheap, easily produced and of superior qualities.

Having thus described my invention, what I claim as new and desire to protect by Letters Patent is:

1. The process of obtaining a composite lubricant comprising distilling acids and aldehydes off from castor oil to eliminate about 6.5% of the whole mass, blowing the 20 resulting product heated to a temperature of from 75° to 150° centigrade with air until the gumminess begins to show a rapid increase with the viscosity greatly increased, and mixing the resulting product with light 25 viscosity mineral lubricating oil in quanti-

ties sufficient to obtain a lubricant of desired viscosity.

2. The process of obtaining a composite lubricant, comprising heating medicinal castor oil in a still at atmospheric pressure 30 until approximately 6.5% of the acids and aldehydes have been driven off, forcing air through the heated residue until the gumminess of the mass begins to increase rapidly, and mixing the heavy resulting product with light grades of mineral oil lubricant in the proportions desired.

3. The process of obtaining a composite lubricant comprising distilling off from castor oil the acids and aldehydes to about 40 6.5% of the mass, blowing the residue with air until a point of rapid increase of gumminess is reached and mixing the resulting product with lighter mineral oil lubricants in the manner set forth.

In testimony whereof I hereunto affix my signature this the 7th day of July, A. D. 1922.

DEMPSEY KEMP DODGE.